

Dec. 31, 1929.

H. L. COXEY

1,741,615

HOT TOP FOR INGOT MOLDS

Filed June 25, 1927

3 Sheets-Sheet 1

Fig. 1.



Fig. 3.



Fig. 4.



Fig. 2.



By

Horace L. Coxey Inventor

Murra Kline.

Attorney

Dec. 31, 1929.

H. L. COXEY

1,741,615

HOT TOP FOR INGOT MOLDS

Filed June 25, 1927

3 Sheets-Sheet 2

Fig. 5.



Fig. 6.



Fig. 7.

Inventor

Horace L. Coxey

Munson Crane

By

Attorney

Dec. 31, 1929.

H. L. COXEY

1,741,615

HOT TOP FOR INGOT MOLDS

Filed June 25, 1927

3 Sheets-Sheet 3



Fig. 8.

Fig. 9.



Fig. 10.

INVENTOR.  
*Horace L. Coxey*  
BY *William H. Lane*

ATTORNEY.

## UNITED STATES PATENT OFFICE

HORACE L. COXEY, OF MASSILLON, OHIO

## HOT TOP FOR INGOT MOLDS

Application filed June 25, 1927. Serial No. 201,362.

The invention relates to what are known in the art as hot tops, hot feeders, or sink heads for ingot molds.

The broad object of the invention is to prevent piping of the steel in the ingot mold, due to contraction in the steel caused by more rapid cooling on the outside than on the inside. Other hot tops have been designed with this broad object in view, but in most instances they have not proved satisfactory on account of various factors, such as the expense of a complicated structure, the difficulty of using certain types of hot tops where ordinary unskilled labor is employed; and the fact that with certain proposed types of hot tops unsound ingots are produced due to a slight porosity at the junction between the hot top and the ingot.

The present invention has been designed in view of the defects of previous hot tops, and the object of this invention is to produce a simple form of device, which may be manufactured at relatively low cost, which is light in weight, requires no skill on the part of the workman using the same, which will adequately prevent piping, which insures a sound ingot at the junction between the ingot and hot top, and which permits a material saving of material, ordinarily wasted in the usual form of hot top.

The invention is in some respects a combination of certain desirable features individually old in the art, into a single structure, for the purpose of eliminating the disadvantages possessed by the prior structures; and for producing a single device which will accomplish new and improved results. Certain other features of the invention are in themselves broadly novel, in addition to their cooperation with the other elements of the device to produce the improved combination.

With these objects in view, the invention will be more fully understood by a brief reference to the conditions which are present in the pouring of steel into ingot molds.

When molten steel is poured into ingot molds, what is known in the art as a hot top feeder or sink head, is employed for feeding the molten metal into the voids of the ingot, caused by the shrinkage of the solidifying

steel in the mold. This hot top should be separate from the ingot mold, but should be light and cheap, and readily applied to the mold. The steel is poured until it fills the mold and the hot top. When the ingot has hardened it is removed from the mold, and that portion which was in the hot top becomes waste material, and is sheared off and discarded as "scrap." It is important that the steel in the ingot be sound, and free from flaws or piping, and that it is free from porosity at the junction between the hot top and the mold. In order that the material in the ingot mold be sound it is necessary that considerable pressure be exerted upon it from above, and that the cooling be slow and uniform throughout. Increase in pressure may be had by increasing the height of the hot top, but with the ordinary form of hot top, such increase in height would result in considerable additional loss of metal as scrap, and furthermore with high hot tops of ordinary construction there is an increased tendency toward uneven cooling with the resulting piping. Consequently it is necessary to strike a balance between the desirability of having as much pressure as possible and the disadvantages following from too high a hot top. The present invention permits of a high hot top, with less waste and less piping than in previous devices.

In order to accomplish the desired results, the present device possesses certain characteristic features which will now be described.

The hot top is made of a non-metallic porous insulating material with a smooth inner coating of refractory material to prevent the metal from eating into the walls of the hot top. The insulating material of which the hot top is composed is highly porous, and is preferably made by mixing cork or other carbonaceous material with a refractory mass, molding in the desired form, and burning until a strong permanent bond is formed. The cork or other carbonaceous material burns away in the kiln leaving still air spaces in the form of pores, which, with the insulating material of which the device as a whole is composed, forms a non-conductor of heat. In place of cork, finely divided charcoal, peat

and other carbonaceous material may be employed. The relative proportions of the carbonaceous material and refractory material may be varied as desired, according to the desired degree of porosity of the finished product.

To further augment this insulating capacity, dead air chambers are molded within the walls of the insulating material. With this material no provision is necessary for sealing air or for releasing pressure as the pores in the material itself automatically take care of that. A hot top so formed is lighter than any previously known, on account of the material and construction, and thus allows easier handling, which is an important factor, when it is considered that great numbers of them must be handled daily in the steel mills. No metallic casing is used, and thus heat losses due to conduction are avoided and the weight of the metal is eliminated.

In order to produce the maximum pressure upon the ingot with the least waste of scrap material in the hot top, the hot top is formed with a base of substantially greater area than the area at the upper portion thereof. The saving in metal due to this change in construction, by reason of the difference between the top and bottom areas amounts to from 20 to 25% for the smaller hot tops and more in the hot tops used for larger molds. This saving in metal is very considerable and the saving in metal over the ordinary mold is approximately equal to the cost of the hot top, for one single casting operation. On account of this construction it is obvious that the height of the hot top could be increased without having to pour more metal in the hot top for a given ingot mold than is used in the ordinary type of hot top and such increase of height would, on account of the added pressure produce a sounder ingot than is produced according to the present practice, the ordinary casting showing a slight porosity at the junction between the hot top and the ingot, this porosity being evident when that portion of the ingot is etched with a suitable reagent.

The combined device, with its larger base than top, and with its walls composed of light, porous insulating material, having a dead air space molded therein, will keep the metal hot and in liquid condition for a long period of time, and thus the metal will feed freely from the hot top into the ingot mold as the metal in the ingot mold is shrinking down, and combined with the increased pressure due to the greater height of the hot top permissible when using this type of device, the construction and composition of the hot top as a whole insure a sound ingot in which piping and flaws are eliminated and in which there is a minimum loss in the form of scrap.

While it will be obvious that the invention is not limited to particular details of construc-

tion, a more complete understanding of the invention may be had by reference to the accompanying drawings in which are shown several illustrative embodiments of the invention.

In the drawings:—

Fig. 1 is a central vertical section showing one form of hot top, a portion ingot mold being shown fragmentarily.

Fig. 2 is a top plan view of the same.

Fig. 3 is a bottom view.

Fig. 4 is a horizontal sectional view on line 4—4 of Fig. 1.

Fig. 5 is a vertical sectional view similar to Fig. 1, but showing a modification.

Fig. 6 is a horizontal section on line 6—6 of Fig. 5.

Fig. 7 is a bottom view.

Fig. 8 is a vertical section showing a third modification.

Fig. 9 is a horizontal sectional view on line 9—9 of Fig. 8.

Fig. 10 is a view similar to Fig. 9, but showing a modification in which the hot top is circular in cross section rather than square as in Figs. 8 and 9.

Referring first to Figs. 1—4 inclusive, the reference numeral 10 denotes the usual metal ingot mold which in this instance is rectangular in cross section. Metal is poured into the ingot mold through a hot top 11 which is removable, and of light weight, and provided with handles 12 to facilitate lifting the same into position upon the mold. The hot top is of porous, insulating material, preferably produced by mixing cork or other carbonaceous material with refractory material, molding the same into form, then burning out the carbonaceous material at the same time that the mass is hardened into permanent form. In this manner the walls are made porous, the pores being filled with still air, which provides excellent insulation. In order to increase its insulating capacity, and to further lighten the material the walls are provided with a plurality of large air spaces 13 within the walls themselves, and substantially surrounding the entire mass of hot steel within the hot top. In this manner very light weight is secured, accompanied by highest efficiency from the point of view of insulation.

To form the air spaces 13, a hot top form or mold is placed on a steel plate with the small end of the mold resting on the plate. This leaves the large end of the mold up, ready to be filled with suitable material and rammed. The first operation consists in ramming approximately one inch of material in the mold. Then strips or patterns of the proper size chambers are placed inside, and rammed to form the air spaces. The patterns are then withdrawn and the spaces left are covered with card board or heavy paper to maintain the air spaces. The remaining material for forming the hot top is supplied

and rammed. After the hot top is formed, it is hardened by suitable heating, this heating operation serving to burn out the carbonaceous material within the mass, of which the hot top is composed.

5 It has been found that the less material used in the hot top, and the thinner the walls, where made of suitable insulating material, the less piping occurs. On the inside of the hot top, as at 14, an inner layer of smooth, non-porous refractory insulating material is preferably employed. This serves two functions, namely, to prevent the steel from permeating the pores of the hot top, and, second, to prevent 10 the outside air from circulating into the interior of the hot top, the lining thus cooperating with the dead air space 13 to produce more efficient insulation. Such hot top may be very thin and light indeed and is easily 15 handled.

As shown, the hot top is rectangular in cross section, and the area across the base, as at 15, at the top of the ingot mold is much less than at 16, which is the limit to which steel is 20 poured, this being at the upper limit of the dead air spaces 13.

A suitable flange 17 extends into the ingot mold to prevent access of air at the junction between the hot box and ingot mold, and a 25 flanged seat 18 is formed at the base of the hot top, which rests upon the wall of the mold 10. This construction is simple and cheaply manufactured and is very efficient in preventing piping.

30 The construction shown in Figs. 5-7 is similar to that already described except that the hot top is in the form of a frustum of cone, and is adapted for use on a circular mold. It will also be noted that an outwardly extending 35 flange 19 is provided to serve as a seat for the hot top upon the mold 10, and the dead air spaces 13 are circularly arranged.

In Figs. 8, 9 and 10, the upper area of the hot top is substantially smaller than the lower 40 area, as in the previously described forms, but in this case, instead of the walls flaring uniformly outwardly from top to bottom, the walls are vertical for a substantial portion of their height, and flare abruptly outwardly 45 near the base as shown at 20 in Fig. 8. In Figs. 8 and 9, the hot top is square in section, while in Fig. 10 it is circular. Otherwise, the 50 two constructions are the same.

The invention has been described in considerable detail, for the purpose of illustration, but it will be evident that it is capable 55 of many modifications within the scope of the appended claim.

60 The hot tops are in each case provided with flat covers made of insulating material and provided with flanges projecting downwardly over the upper edge of the hot tops, these 65 covers being designed to keep in the heat and to help keep the metal liquid.

What I claim is:—

A hot top for ingot molds having a wall composed of insulating material having pores therein communicating with the outer surface of the hot top and relatively large air 70 spaces formed within said wall communicating with the outer atmosphere through said pores and sealed from the interior of the hot top by means of smooth non-porous refractory material.

In testimony whereof I affix my signature.

HORACE L. COXEY.

80

85

90

95

100

105

110

115

120

125

130